

## UNITED STATES PATENT OFFICE

DANIEL HARVEY MELOCHE, OF NEW YORK, N. Y., ASSIGNOR TO AMERICAN RADIATOR COMPANY, OF NEW YORK, N. Y., A CORPORATION OF NEW JERSEY

## CAST-METAL PIPE AND METHOD OF MAKING THE SAME

No Drawing.

Application filed May 17, 1928. Serial No. 278,626.

My invention relates to new and useful improvements in cast metal pipe and a method of making the same, and more particularly contemplates as a new article of manufacture 5 a cast iron pipe having pronounced features of novelty over any previous cast iron pipe of which I am aware, and which will be capable of being machined, cut, or threaded in a manner and to an extent which was impossible in cast iron pipe hitherto known.

It is well known that cast iron pipe as made previous to my invention, was hard and brittle, comparatively easy of fracture, and, therefore, could not be machined, cut, or 15 threaded by ordinary pipe cutting or threading tools. Furthermore, cast iron pipe as previously known, being hard and brittle as compared to steel and wrought iron pipe, was not capable of being cut to length or 20 threaded with standard tools in order to render the same capable of use with ordinary threaded couplings such as are commonly used to join lengths of steel or wrought iron pipe, and it was necessary either to employ 25 packed joint coupling elements made separate from the pipe, or cast the elements of such couplings integral with the pipe. It was also necessary to cast the pipe with a metal line or wall which was thicker, as compared with steel and wrought iron pipe, in 30 order to give the cast pipe sufficient strength to withstand fracture which might result from bursting or tensile transverse breaking strains. The cast iron pipe as previously 35 known, had little or no resiliency transverse to its longitudinal axis, as compared to steel or wrought iron pipe, and therefore was liable to break when subjected to transverse bending strains or deflections.

40 It is therefore one of the objects of my invention to provide a cast iron pipe having characteristics which will render it capable of being readily machinable, or cut, or threaded by standard tools such as are ordinarily employed in the cutting or threading of steel or wrought iron pipe.

45 A further object is to provide a cast iron pipe which will have a metal line substantially the same as commercial steel or wrought 50 iron pipe of a corresponding outside diam-

eter, and which will withstand transverse or bursting strains far in excess of heretofore known cast iron pipe, and to an extent favorably comparable with steel and wrought iron pipe.

55 A further object is to provide a cast iron pipe having characteristics attaining the objects above mentioned, which will withstand erosion or corrosion effects, and be of long life in use as compared with ordinary known 60 gray cast iron pipe and commercial steel or wrought iron pipe.

65 A further object is to provide a novel method or process for producing a cast iron pipe capable of having the novel characteristics herein set forth.

70 According to my invention I cast the pipe from molten alloy metal having substantially the following analysis by percentages at the cupola spout:

|                                            |              |
|--------------------------------------------|--------------|
| Silicon                                    | 2.25 to 2.50 |
| Manganese                                  | .60 to .80   |
| Phosphorus                                 | .20 to .30   |
| Sulphur, below                             | .1           |
| Combined carbons                           | .50 to .60   |
| Graphitic carbon, less than                | 2.75         |
| Total carbons                              | 3.30 to 3.35 |
| Nickel                                     | .10 to .15   |
| Chromium                                   | .20 to .30   |
| Iron substantially the balance to make 100 | 80           |
| per cent.                                  |              |

85 It will be understood that the analysis of the finished casting is preferably within the limits above given, but the range of percentages may be slightly above or slightly below the maximums and minimums given, so as to be substantially of the percentages given and within proportions relatively which will produce pipe having the novel characteristics 90 herein described. The alloy iron of the analysis above given may be produced in a cupola of any known structure, the ingredients or elements being selected and proportioned relative to each other, so that the molten metal 95 at the cupola spout will have the analysis substantially as above given. The chromium and nickel may be supplied, if desired, by the use of Mayari pig-iron as a part of the cupola charge, for example Mayari pig-iron 100

containing approximately 1% of nickel and 2% of chromium, together with traces of vanadium, cobalt and titanium. In the event that Mayari pig-iron be not employed as part of the charge, I add nickel and chromium, or elements containing the same, in proper proportions to produce the spout analysis given. In any event it is necessary to employ a charge which will contain a relatively high silicon percentage and a low phosphorous percentage as given, so that the total carbons will be maintained at or within the limits stated, and a high proportion of the total carbons will be graphitic carbon and a low proportion will be combined carbons. The percentage of phosphorous must be low enough so that the metal will not be made hard or brittle, and therefore unduly resistant to standard cutting and threading tools. By cutting and threading tools I mean such tools as are ordinarily employed in the trades for cutting and threading steel or wrought iron pipe.

The charge in the cupola or melting furnace is heated to a temperature above that ordinarily employed in producing gray cast iron for making pipe as hitherto known, which insures that graphitic carbon will be precipitated from the molten metal to as great an extent as is practically possible, and further insures that the graphitic carbon precipitated will be in a finely divided state or minute particles, as distinguished from the comparatively large flakes, as the same usually appear in micrographs of ordinary gray cast iron. Preferably, the metal is heated in the cupola to such a temperature that the metal at the spout will be at a temperature of approximately 2700° F. to 2800° F., which is well above the spout temperature in the case of ordinary gray cast iron when used for casting pipe, which is normally about 2600° F.

In casting the pipe, I preferably employ a suitable mold or flask structure lined with a sand mold which is dried or baked, and also use a suitable core of dried or baked sand, the inside diameter of the mold and the outside diameter of the core being such as to produce pipe having a desired metal line or wall thickness. The sand mold and the sand core are heated by any suitable means, for example, in a suitable oven before the casting is poured, so that the mold and core will be at a temperature of approximately 400° F. when the metal is poured into the mold, and the metal is poured into the mold and around the core while the molten metal is at a temperature of approximately 2500° F. By pouring the metal at the temperature mentioned into the heated sand mold while the latter is at a temperature of 400° F. approximately, the graphite or graphitic carbon in the metal will be maintained in a finely divided state or minute par-

ticles, and the other elements in the metal will not become segregated during the pouring of the casting and during the cooling or setting thereof, thereby producing a uniform casting. It is important that the charge be heated in the cupola to a temperature high enough to cause segregation and precipitation of the carbon as graphitic carbon in a finely divided condition in the ultimate pipe casting, and also to cast the pipe in a preliminarily heated mold in order that the precipitated graphitic carbon will be maintained in the finely divided condition or minute particles, as this heating not only serves to reduce the percentage of combined carbons, and thereby enhance the machinability of the pipe, but the finely divided condition of the graphite reduces the corrodibility of the casting by elements to which it may be subjected when in use. The iron content of the casting which completes the formula heretofore given, is substantially all in the form of ferrite, or its compounds, so that the pipe may be readily cut or threaded with such tools as are ordinarily employed for cutting and threading steel and wrought iron pipe, and such cutting or threading will not be attended with danger of fracture, as is the case with hitherto known cast iron pipe made from gray iron.

It will be noted that according to the analysis above given, the manganese is in the proportion given as a safety factor to reduce the sulphur content of the resultant iron, and prevent any such excess of sulphur that might tend to make the iron brittle. The carbon and silicon proportions as above given are maintained so as to produce an iron which will have the desired ductility. The nickel and chromium act to accelerate the precipitation of the carbon from solution, the precipitation of the carbon being, as stated above, in the form of graphite in a finely divided state, and being a large proportion of the total carbons, results in a casting which will be of the desired ductility and such as may be readily cut or threaded with standard tools.

Pipe made according to my invention will be found very resistant to corrosion and erosion, and therefore of considerably greater life than commercial steel or wrought iron pipe when used under conditions which would tend to erode or corrode the same, for example, my pipe as herein described can be satisfactorily used for acid lines of chemical plants, whether the acid be hot, cold, weak or concentrated, and will stand up for a long period of time, whereas commercial steel and wrought iron pipe would be destroyed in a comparatively short time. My pipe also has long life in oil refinery systems, in acid sludge lines, contact plants, condenser boxes, and run-down lines, where any commercial steel or wrought iron pipe would be compara-

tively short lived, due to erosion or corrosion by the acid content of the conveyed liquid or vapor.

Pipe made according to my invention may be and preferably is cast with a metal line or wall thickness substantially the same as commercial steel or wrought iron pipe of the same outside diameter—for example, pipe of 1.9 inches outside diameter may have a metal line of substantially .20 inches; pipe having an outside diameter substantially 2.375 inches may have a metal line of substantially .218 inches; pipe having an outside diameter of 2.875 inches may have a metal line of substantially .276 inches; pipe having an outside diameter of 3.50 inches may have a metal line of .30 inches, and pipe having an outside diameter of 4.50 inches may have a metal line of .337 inches, these metal lines being substantially the same as high quality, extra strong commercial steel or wrought iron pipe. Pipe made according to my invention will have high resistance against breakage under hydraulic internal pressure test—for example, pipe having an outside diameter of 1.9 inches and a metal line of .20 inches, will withstand an internal pressure test of substantially 4000 pounds per square inch before breakage; the pipe of 2.375 inches outside diameter will withstand a test of approximately 4050 pounds per square inch before breakage; the pipe of 3.50 outside diameter will withstand a pressure test of approximately 3800 pounds per square inch before breakage, and the pipe of 4.50 outside diameter will withstand a pressure test of approximately 3000 pounds per square inch before breakage, which compares favorably with the best commercial steel or wrought iron pipe.

The pipe will also withstand tensile strength tests of approximately 30,000 pounds or over, and is resilient, in that it may be deflected to a considerable extent, without breakage, transversely to its longitudinal axis—for example, in the case of the 1.9 inch outside diameter pipe mentioned and 6 feet in length, will come back to perfect alinement after at 1½ inch deflection from its longitudinal axis; and such pipe will withstand a deflection of approximately 1¾ inches before breakage; the pipe of 2.375 inches outside diameter will come back to alinement after a deflection of 1½ inches, and will withstand a deflection of 1½ inches before breakage; the pipe of 3.5 inches outside diameter can be deflected ¾ of an inch and will withstand a deflection of 1½ inches before breakage; and the pipe of 4.5 inches outside diameter may be deflected ½ inch and will withstand deflection up to ½ of an inch before breakage, it being understood that the pipes of the outside diameters just mentioned were all tested at a 6 foot length and had the metal lines above given respec-

tively. In these tests each length of pipe was supported 3 inches from each end, and the force was applied at the center. The pipe also is capable of withstanding large, transverse breaking strains—for example, it will have a transverse strength of from 3000 to 4000 pounds when tested by a standard arbitration bar.

The pipe also has a further and important advantage that it may be cast to standard lengths in the foundry, and either threaded at the foundry by such tools as are ordinarily used for threading commercial steel and wrought iron pipe, or the lengths as cast may be afterwards cut in the field by ordinary pipe cutting tools at any desired point and to a desired length, and then be threaded by ordinary tools such as are employed by plumbers and pipe fitters.

What I claim and desire to secure by Letters Patent of the United States is:—

1. As a new article of manufacture, a pipe made of a casting of alloy iron, which is ductile and capable of being cut or threaded at any point in its length by standard tools such as are employed for cutting and threading steel and wrought iron pipe, said pipe also being transversely resilient substantially to the same extent as steel or wrought iron pipe of the same dimensions, said pipe being highly resistant to erosion and corrosion.

2. As a new article of manufacture, a cast pipe made of cast iron alloy comprising silicon 2.25% to 2.50%; phosphorus .2% to .3%; manganese .6% to .8%; sulphur below .1%; combined carbons .5% to .6%; graphitic carbon not to exceed substantially 2.75%; total carbons from 3.30% to 3.35%; and an accelerator for precipitation of graphitic carbon; and iron approximately sufficient to complete the 100%, said pipe being ductile and capable of being cut or threaded at any point along its length by means of tools such as are used for cutting or threading steel or wrought iron pipe, and being resilient on its longitudinal axis.

3. As a new article of manufacture, a cast pipe made of a cast iron alloy comprising silicon 2.25% to 2.50%; manganese not more than .8%; phosphorus not more than .3%; sulphur not more than .1%; combined carbons not more than .6%; graphitic carbon not to exceed substantially 2.75%; total carbons not more than 3.35%; nickel approximately 1% to 15%; chromium approximately 2% to 3%; and iron approximately sufficient to complete the 100%; said pipe being ductile and capable of being cut or threaded at any point of its length by means of tools such as are used for threading and cutting steel or wrought iron pipe, and being resilient on its longitudinal axis.

4. As a new article of manufacture a cast pipe made of a cast iron alloy comprising silicon 2.25% to 2.50%; manganese .6% to

8%; phosphorus .2% to .3%; sulphur below .1%; combined carbons .5% to .6%; graphitic carbon less than 2.75%; total carbons from 3.30% to 3.35%; nickel .1% to .15%; chromium .2% to .3%; and ferrite approximately sufficient to complete the 100%; said pipe being ductile and capable of being cut and threaded at any point of its length by means of tools such as are used for cutting or threading 10 steel or wrought iron pipe, and being resilient on its longitudinal axis.

5. A process of producing cast iron pipe, which cast iron pipe will be ductile and capable of being cut or threaded at any point in its length by tools such as are used for cutting or threading steel or wrought iron pipe, which comprises producing a molten iron containing silicon 2.25% to 2.50%; manganese not more than .8%; phosphorus not more than .3%; sulphur not more than .1%; combined carbons not more than .6%; graphitic carbon not to exceed substantially 2.75%; total carbons not more than 3.35%; an accelerator for precipitation of the graphitic carbon; and iron approximately sufficient to complete the 100%; said molten iron being heated to a temperature causing the precipitation of the graphitic carbon in a finely divided condition, and casting the said molten metal in a sand mold heated to a temperature maintaining the finely divided state of the graphitic carbon and preventing segregation of the elements.

6. A process of producing cast iron pipe, which cast iron pipe will be ductile and capable of being cut or threaded at any point in its length by tools such as are used for cutting or threading steel or wrought iron pipe, which comprises producing a molten iron containing silicon 2.25% to 2.50%; manganese not more than .8%; phosphorus not more than .3%; sulphur not more than .1%; combined carbons not more than .6%; graphitic carbon not to exceed substantially 2.75%; total carbons not more than 3.35%; an accelerator for precipitation of the graphitic carbon; and iron approximately sufficient to complete the 100%; said molten iron being heated to a temperature of from approximately 2700° F. to approximately 2800° F., thereby causing the precipitation of the graphitic carbon in a finely divided condition, and casting the said molten metal in a sand mold heated to a temperature maintaining the finely divided state of the graphitic carbon and preventing segregation of the elements.

7. A process of producing cast iron pipe, which cast iron pipe will be ductile and capable of being cut or threaded at any point in its length by tools such as are used for cutting or threading steel or wrought iron pipe, which comprises producing a molten iron containing silicon 2.25% to 2.50%; manganese not more than .8%; phosphorus not

more than .3%; sulphur not more than .1%; combined carbons not more than .6%; graphitic carbon not to exceed substantially 2.75%; total carbons not more than 3.35%; an accelerator for precipitation of the graphitic carbon; and iron approximately sufficient to complete the 100%; said molten iron being heated to a temperature of from approximately 2700° F. to approximately 2800° F., thereby causing the precipitation of the graphitic carbon in a finely divided condition, and casting the said molten metal in a sand mold heated to substantially 400° F. to thereby maintain the finely divided state of the graphitic carbon and preventing segregation of the elements.

8. A process of producing cast iron pipe, which cast iron pipe will be ductile and capable of being cut or threaded at any point in its length by tools such as are used for cutting or threading steel or wrought iron pipe, which comprises producing a molten iron containing silicon 2.25% to 2.50%; manganese not more than .8%; phosphorus not more than .3%; sulphur not more than .1%; combined carbons not more than .6%; graphitic carbon not to exceed substantially 2.75%; total carbons not more than 3.35%; an accelerator for precipitation of the graphitic carbon; and iron approximately sufficient to complete the 100%; said molten iron being heated to a temperature of from approximately 2700° F. to approximately 2800° F., thereby causing the precipitation of the graphitic carbon in a finely divided condition, and casting the said molten metal in a baked sand mold heated to substantially 400° F. to thereby maintain the finely divided state of the graphitic carbon and preventing segregation of the elements.

In testimony whereof I have hereunto signed my name.

DANIEL HARVEY MELOCHE.

110

115

120

125

130